

July 10, 1923.

1,461,018

P. A. E. ARMSTRONG

METHOD OF MAKING TUBULAR BODIES

Filed Feb. 3, 1919



Fig. 1



Fig. 2

INVENTOR  
P. A. E. Armstrong  
BY  
H. H. Dyke  
ATTORNEY

Patented July 10, 1923.

1,461,018

# UNITED STATES PATENT OFFICE.

PERCY A. E. ARMSTRONG, OF LOUDONVILLE, NEW YORK.

## METHOD OF MAKING TUBULAR BODIES.

Application filed February 8, 1919. Serial No. 274,639.

To all whom it may concern:

Be it known that I, Percy A. E. Armstrong, a subject of the King of Great Britain, and a resident of Loudonville, county of Albany, and State of New York, have invented certain new and useful Improvements in Methods of Making Tubular Bodies, of which the following is a specification.

10 This invention relates to an improved process of making tubular bodies such as hollow drill rod and the like.

Heretofore in making such tubular members a billet has been provided with a longitudinal bore, as by drilling, and after the bore has been formed a core has been introduced into said bore and the billet and core elongated and reduced in cross-section, as by rolling, and the core removed.

20 According to the present invention the core is placed within an ingot mold and the material from which the elongated tubular body is to be formed, as steel in the case of making hollow drill rod, is introduced there-  
25 in around the core while in molten state, and when it has solidified with the core in place therein the ingot and core are subjected to treatment for elongation and reduction of cross-section, as by rolling, after  
30 which the core is removed, leaving the tubular body desired to be produced.

The ingot, with the core in place therein, may be rolled before being cooled down from its casting heat to below rolling temperature, or it may be further cooled and re-heated for rolling, as will be readily understood.

35 Cores of various kinds may be used, so long as same are adapted for removal after rolling. For example, the core may be substantially entirely of refractory material, such as finely divided talc, magnesite or other suitable materials which are substantially infusible at the temperature employed.

45 In such case the core ends are preferably sealed in place, as by welding over or the like, before rolling; or an all metal core with a surface layer of non-welding material, such as aluminum oxide, lime or the like, may be employed, and various other forms of core may be used and same may be in one part or may be in two or more parts.

50 Preferably, a core such as is illustrated in the accompanying drawing is used, comprising a metallic interior member which may, for convenience, be termed a rod, and

an outer substantially thick surrounding layer of refractory material, such as talc, dead burned magnesite or other suitable material which is substantially infusible at the 60 temperatures to which it is subjected. After rolling the drill rod or other tubular body may be cut or broken into commercial lengths, and the core removed either before or after such division into lengths. If the 65 core end projects as shown in the drawing it may conveniently provide a head, after rolling, to fasten to for core pulling, and the other end may be cut or broken off to remove any malformed portion. The follow- 70 ing end of the rod, which is pulled through and comes out last, may be deformed, as by striking with a hammer or other tool, and the battered end may serve for breaking up the layer of refractory material, which can 75 then be readily removed. Pushing may be resorted to for partial or entire removal of the core rod when desired.

In the drawing, Fig. 1 is a diagrammatic, longitudinal, sectional view of an ingot 80 mold with a core and an ingot being cast therein. Fig. 2 is a plan view showing a centralizing holder for the core. In said drawing the ingot mold, which may be of any usual or desired form is represented at 85 10. The core is represented at 11 and comprises a metallic interior member 12 and a substantially thick surrounding layer 13 of refractory material. 14 designates the molten material from which the tubular 90 body is formed, as steel for making hollow drill rod.

The core may be centralized in any de- 95 sired manner, as by providing a recess or socket 15 to receive the bottom end thereof and by applying suitable holding means to the upper end 16 of the core, or in other ways. In the form shown a crossbar 17 is illustrated for supporting the upper end of the core centrally of the mold. It has an 100 opening 18 for the core and has an extended base 19 which fits within the mold and serves to centralize the opening 18 and thereby the core. The leg 20 bears against the mold on the side opposite the base 19. 105 By making the supporting member in the form shown, the core may be held stationary in properly centralized position, and at the same time there is ample room for pouring the molten metal in place. Other forms of 110 centralizing means may of course, be used. The cast ingot with the core in place therein,

after removal from the mold is treated for elongation and reduction of cross-sectional ingot and core, as by rolling or the like operation, and the core removed. When the 5 core consists of a central rod or the like surrounded with refractory material, the rod is first removed and thereafter the refractory material cleaned out.

It will be seen that among the advantages 10 secured by the process of the present invention are these:

It results in a substantial saving of work, time and material. It entirely dispenses with the formation of the bore in a billet as 15 a separate operational step and with any necessity for fastening the core in place against relative movement after insertion into a previously bored billet. It eliminates any danger of injuring the core or its 20 surface, which may be encountered when inserting same into a previously formed billet bore.

It is to be understood, however, that the 25 type of core shown is for illustration only and that cores and weld-preventing materials of various kinds may be resorted to,

so long as the ingot is formed by casting around the core, and further, that while my invention has been described more particularly in connection with making hollow 30 drill rod, it is applicable to making tubular bodies generally.

I claim:

1. The process of making tubular bodies such as hollow drill rod and the like which 35 consists in casting an ingot around a core, treating the ingot and core for elongation and reduction of cross-section, as by rolling and removing the core.

2. The process of making tubular bodies 40 such as hollow drill rod and the like, which consists in casting an ingot around a core comprising a metal rod and a substantially thick surrounding layer of refractory material, treating the ingot and core for elongation and reduction of cross-section, as by 45 rolling, removing the core rod, and removing the refractory material.

In testimony that I claim the foregoing, I have hereto set my hand, this 31st day of 50 January, 1919.

PERCY A. E. ARMSTRONG.